# EUROPEAN PATENT SPECIFICATION

(11) **EP 0 060 354 B1**
(45) Date of publication and mention of the grant of the patent: **31.07.1985**
(21) Application number: 81301043.6
(22) Date of filing: 12.03.1981
(51) Int. Cl.: C10L 9/02

(54) **Method of treating coal to remove sulphur and ash**
Verfahren zum Entfernen von Schwefel und Asche aus Kohle
Procédé d'élimination du soufre et des cendres de charbon

(43) Date of publication of application: 22.09.1982
(73) Proprietor: Carson, Dennis M., Cincinnati Ohio 45202 (US); Feldkamp, Joseph F., Jr., Cincinnati Ohio 45202 (US)
(72) Inventor: Brown, George E., Jr., Cincinnati Ohio 45241 (US)
(74) Representative: Allen, Oliver John Richard

## Description

There exists in the United States a large quantity of coal which cannot be economically used as a fuel because of its high sulfur content. Environmental laws are such that it is enconomi- cally unfeasible to burn a high sulfur content coal because of the expensive antipollution equipment required.

High sulfur coal, i.e., about 3%, exists in unmined form and also in the form of already mined coal that has been discarded, i.e., refuse coal. Refuse coal usually consists of fines which result from the processing of coal. More particularly, when coal is mined it is normally crushed and washed and the washings are generally dumped and used as land fill or dumped into a lake or stream. In the latter case, over a period of time, the pond or stream becomes almost completely filled with the finely powdered coal. Not only is this is a significant waste of coal but it is injurious to the lakes and streams. Many lakes have become "dead" lakes dueto this disposal of waste coal. The ash content of such refuse coal, i.e., above 20% by weight, also makes it economically unattractive to attempt to utilize it.

There also exist in the United States substantial. deposits of unmined or virgin coal having a high sulfur content. In order to burn such coal in industry it would be necessary to spend substantial amounts of money for air pollution equipment. Therefore, this high sulfur content coal is not being mined.

The need to effectively utilize energy while at the same time protecting our environment faces many other industries as well, the steel industry being another example. The disposal of waste materials from steel making processes in an economically feasible, environmentally suitable manner is frequently a significant problem. For example, in the processing of steel an acid solution (pickle liquor) is used to treat the product. The resultant solution consisting of an acid, iron compounds, contaminants, etc. (collectively referred to hereinafter as spent pickle liquor) must be disposed of.

In accordance with one aspect of the invention, a method of treating pulverised coal to remove sulphur comprises adding pickle liquor to the coal, subsequent adding to the coal of a mixture of water with chlorine gas added thereto, the amount of pickle liquor and chlorine gas being sufficient to provide a mixture having a pH of less than about 3, and physically separating the coal from the mixture.

The present invention is applicable to high sulphur, high ash refuse or virgin coal. In one form of the present process, coal, crushed to about 1/4 by 0 size (that is 1/4 inch down to 325 Tyler mesh in size6.35 to 0.04x10-²m) is first treated with spent pickle liquor. Thereafter it is subjected to a strong acidic oxidizing agent. More particularly, the acidified coal mixture is treated with a mixture of chlorine gas dissolved in water. Thereafter coal and ash are separated through the use of water and gravity. Following this, the acid solution remaining is treated with lime and the precipitate which contains various sulfur compounds is discarded. These sulfur compounds exists in such a state that they are not injurious to our environment when discarded and in fact have a beneficial effect on dead lakes.

In accordance with another aspect of the invention, a method of removing ash and sulphur from coal wherein sulphur is present comprises forming a coal and water mixture from pulverized coal and a minor amount of water, treating the mixture with chlorine gas in an amount sufficient to convert the sulphur to a sulphur containing acid(s), physically separating ash and coal from the mixture, treating the remaining mixture containing the sulphur containing acid(s) with lime whereby the sulphur is precipitated as calcium salts, and physically separating the calcium salts.

In this alternative form of the present invention only a minor amount of water is added to the pulverized coal, preferably in the form of steam, and the mixture is treated with chlorine gas.

The process of this invention can be effectively practised on any high sulphur content coal. In its most useful application it is practised on refuse coal that at the present time has no utility. After treatment the refuse coal contains less than about 1% sulphur, has about 5-6% ash, has about 14,000-14,500 British thermal unit (btu) per pound (3:26-3.37x104 J/kg), and is processed into easily handled pellets. In contrast, before processing the refuse coal typically contains 2-3% sulphur, 25-30% ash and has a btu per pound content of only 7,500 (1.74x10⁴ J/Kg).

Refuse coal is produced as the result of normal coal mining operations and exists as a result of coal being crushed and washed. Typically it is 1/4 by 0 and discarded as land fill or thrown into a pond, lake or stream. In some instances as much as 20% by weight of the mined coal ends up in the form of heretofore unusable refuse coal.

Various areas of the United States contain large deposits of coal which are basically unusable because of the high sulphur content of the coal. The present process is applicable also to such coal. The only modification required is to pulverize the coal so that it is about 1/4 by 0 as in the case of refuse coal..

In the practice of one embodiment of the process the pulverized coal is first mixed with spent pickle liquor. In the manufacture of iron or steel it is customary to use a pickling acid to remove scale, rust, etc. Most frequently 60° Be' sulfuric acid is employed and this is the preferred form for use in the present invention although other acid pickle liquors may be employed. After use, the spent pickle liquor comprising the acid and various iron compounds such as Fe₂(SO₄)₃₁ FeS0₄.7H₂0 and other contaminants must be disposed of. Obviously, the disposal of such a liquid poses a significant problem from an environmental standpoint.

For some unknown reason the use of spent pickle liquor produces superior results than if the acid itself is used. While it is not completely understood, it is believed that the iron salts present in the spent pickle liquor have a significant effect on the reaction rate.

If only uncontaminated H₂S0₄ is used, the final results in many cases in terms of sulfur removal are inferior and the speed of the reaction is decreased. Moreover, the ability to convert a material that poses such an environmental risk to a safe, useful material able to benefit the environment is an advantage not to be taken lightly. While it is preferred to use spent pickle liquor the acid in unused form may be utilized recognizing, of course, that under some conditions inferior results may be obtained.

The amount of spent pickle liquor mixed with the pulverized coal is somewhat dependent on the sulfur content of the coal. Usually though 2% pickle liquor based on the weight of the coal is sufficient.

It is important to allow the pickle liquor to contact the coal for a brief period of time prior to further processing. In practice 5--10 minutes has been found to be satisfactory. Thereafter, the mixture is introduced into any suitable type of reactor mixture and mixed with about 20% by weight of water. Preferably the water temperature and temperature of the mixture is 80-90°F (26.7-37.2°C). This may require suitable heating or cooling means of conventional design. Into the reactor mixture is introduced chlorine gas. The amount of chlorine required is an amount sufficient to provide a mixture having a pH of about 3 or less. When mixed with the water the chlorine gas provides hydrochloric acid, hypochlorous acid and nascent oxygen.

While it is not completely understood, it is believed that the iron disulphide (iron pyrite) which is present in the coal and which forms the major sulphur containing material is converted into the following iron and sulphur compounds through the following reactions: After the reaction is essentially complete, the ash and coal that are present can be mechanically separated from each other and from the acid solution. One convenient way for doing so consists of introducing the entire mixture into a conically shaped separator of conventional design, where provision is made at the bottom for introducing water. At the top a weir is provided such that material at the surface of the mixture will be transferred out of the separator and into a discharge conduit. The denser heavier coal particles fall to the bottom and are discharged through an outlet. The coal is then dried and preferably pelletized.

To the liquid and water material overflowing the separation is added a sufficient amount of lime to precipitate most of the sulfur as calcium salts, i.e., CaS0₃, CaS, CaS0₄ or other salts of calcium containing sulfur. The amount of lime required is that amount which is required to provide a neutral or nearly neutral pH. Such precipitated salts are thereafter separated and preferably used as fill in coal slurry ponds. If the ponds are not totally filled but if a sufficient amount of the precipitate is added over a relatively short period of time the pond is once again capable of supporting life.

The coal so recovered has less than 6% ash, less than 1% sulfur and a btu content of about 14,000 per pound (3.26x 10⁴ J/kg). The economics of the process are such that refuse coal may be economically reclaimed to provide an excellent energy source.

In the alternative form of the present invention, to the pulverized coal is added a minor amount of water, preferably in the form of steam. The water added is preferably an amount equal to about 10-20 % by weight of the coal. Thereafter, to the mixture is added chlorine gas. Unlike the previous embodiment the chlorine gas is not dissolved in water nor is pickle liquor added to the mixture. Also, the amount of water required is reduced. As in the previous embodiment, the mixture after treatment with the chlorine gas is subjected to the separation step and thereafter to the neutralization step.

## Claims

1. A method of treating pulverized coal to remove sulphur comprising adding pickle liquor to the coal, subsequent adding to the coal of a mixture of water with chlorine gas added thereto, the amount of pickle liquor and chlorine gas being sufficient to provide a mixture having a pH of less than about 3, and physically separating the coal from the mixture.

2. A method as claimed in Claim 1 wherein the mixture remaining after the coal has been removed is neutralised with lime so as to provide a precipitate comprising in substantial part inorganic sulphates.

3. A method as claimed in Claim 1 wherein a substantial amount of ash is physically separated from the mixture simultaneously with the separation of the coal from the mixture.

4. A method as claimed in Claim 3 wherein the mixture remaining after the removal of the coal and ash fractions is neutralised with lime so as to provide a precipitate comprising in substantial part inorganic sulphates.

5. A method as claimed in either Claim 3 or 4 wherein the coal and ash are separated from the mixture through the use of a water flow.

6. A method as claimed in either Claim 2 or 4 wherein the precipitate is used to treat dead bodies of water.

7. A method as claimed in any of the preceding claims wherein the coal is refuse coal.

8. A method of removing ash and sulphur from coal wherein sulphur is present comprising forming a coal and water mixture from pulverized coal and a minor amount of water, treating the mixture with chlorine gas in an amount sufficient to convert the sulphur to a sulphur containing acid(s), physically separating ash and coal from the mixture, treating the remaining mixture containing the sulphur containing acid(s) with lime whereby the sulphur is precipitated as calcium salts, and physically separating the calcium salts.

9. A method as claimed in Claim 8 wherein the coal to be treated is refuse coal and the coal after treatment has less than 6% ash, less than about 1 % sulfur and a BTU content of 14,000 per pound (3.26x10⁴ J/_{K}g).

10. A method as claimed in either Claim 8 or 9 wherein the minor amount of water is 10 to 20% by weight of the coal.

## Patentansprüche

1. Verfahren zur Behandlung von Kohlestaub zur Entfernung von Schwefel, durch Zugabe von Beizflüssigkeit zur Kohle, nachfolgender Zugabe eines Gemischs aus Wasser mit hinzugefügtem Chlorgas zur Kohle, wobei die Beizflüssigkeits-und Chlorgasmenge zur Erzielung eines Gemischs mit einem pH-Wert von weniger als etwa 3 ausreicht, sowie physikalischer Abtrennung der Kohle von dem Gemisch.

2. Verfahren nach Anspruch 1, bei dem das nach Entfernung der Kohle verbleibende Gemisch mit Kalk so neutralisiert wird, dass sich im wesentlichen aus anorgnischen Sulfaten bestehender Niederschlag bildet.

3. Verfahren nach Anspruch 1, bei dem man eine erhebliche Aschenmenge gleichzeitig mit der Abtrennung der Kohle vom Gemisch physikalisch von diesem Gemisch abtrennt.

4. Verfahren nach Anspruch 3, bei dem das nach Entfernung der Kohle und der Aschefraktionen verbleibende Gemisch mit Kalk so neutralisiert, dass sich ein im wesentlichen aus anorganischen Sulfaten bestehender Niederschlag bildet.

5. Verfahren nach Anspruch 3 oder 4, bei dem man die Kohle und Asche unter Verwendung einer Wasserströmung vom Gemisch abtrennt.

6. Verfahren nach Anspruch 2 oder 4, bei dem man den Niederschlag zur Behandlung von stehenden Gewässern verwendet.

7. Verfahren nach einem der vorhergehenden Ansprüche, bei dem man als Kohle Abfallkohle verwendet.

8. Verfahren zur Entfernung von Asche und Schwefel aus schwefelhaltiger Kohle, durch Bildung eines KholelWasser-Gemischs aus Kohlestaub und einer kleinen Menge Wasser, Behandlung des Gemischs mit Chlorgas in einer zur Umwandlung des Schwefels in schwefelhaltige säure (n) ausreichenden Menge, physikalische Abtrennung von Asche und Kohle vom Gemisch, Behandlung des verbleibenden schwefelhaltige Säure(n) enthaltenden Gemischs mit Kalk, wobei der Schwefel in Form von Kalziumsalzen ausfällt, und physikalischer Abtrennung der Kalziumsalze.

9. Verfahren nach Anspruch 8, bei dem man als zu behandelnde Kohle Abfallkohle verwendet und die Kohle nach der Behandlung weniger als 6% Asche und weniger als etwa 1 % Schwefel enthält und einen Heizwert von 3,26x10⁴ J/kg aufweist.

10. Verfahren nach Anspruch 8 oder 9, bei dem die geringe Menge Wasser 10 bis 20 Gew.-% der Kohle ausmacht.

## Revendications

1. Procédé de traitement de charbon pulverisé pour éliminer le soufre comprenant l'addition au charbon d'une liqueur de décapage, suivie d'une addition au charbon d'un mélange d'eau additionée de chlore gaseux, la quantité de liqueur de décapage et de chlore gaseux étant suffisante pour fournir un mélange dont the pH est inférieur à environ 2, ainsi que la séparation physique de charbon du mélange.

2. Procédé selon la revendication 1 caractérisé en ce qu'on neutralise avec de la chaux le mélange restant après l'élimination du charbon, de façon à fournir un précipité comprenant essentiellement des sulfates minéraux.

3. Procédé selon la revendication 1 caractérisé en ce qu'on sépare physiquement du mélange une quantité considérable de cendres simultanément à la séparation de charbon du mélange.

4. Procédé selon la revendication 3 caractérisé en ce qu'on neutralise avec de la chaux le mélange restant après l'élimination des fractions de charbon et de cendres, de façon à fournir un précipite comprenant essentiellement des sulfantes minéraux.

5. Procédé selon la revendication 3 ou 4 caractérisé en ce qu'on sépare le charbon et les cendres du mélange par moyen d'un courant d'eau.

6. Procédé selon la revendication 2 ou 4 caractérisé en ce qu'on utilise le précipité pour traiter des masses d'eaux mortes.

7. Procédé selon l'une quelconque des revendications précédentes, caractérisé en ce que le charbon est du charbon de rébut.

8. Procédé d'élimination des cendres et du soufre du charbon comprenant du soufre caractérisé en ce qu'on forme un mélange charbon et d'eau à partir de charbon pulvérisé et d'une faible quantité d'eau, qu'on traite le mélange au chlore gazeux en quantité suffisante pour transformer le soufre en contenant un acide ou des acides, qu'on sépare physiquement des cendres et du charbon du mélange, qu'on traite avec de la chaux le mélange résiduel contenant le soufre, contenant un acide ou des acides, de sorte que le soufre se précipite sous forme de sels de calcium.

9. Procédé selon la revendication 8 caractérisé en ce que le charbon à traiter est du charbon de rébut et en ce qu'après traitement le charbon contient moins de 6% de cendres, moins d'environ 1% de soufre, et possède un pouvoir calorifique de 14.000 BTU par livre (3,26.10⁴ J/kg).

10. Procédé selon la revendication 8 ou 9, caractérisé en ce que le faible quantité d'eau représente 10 à 20% en poids du charbon.
